# EUROPEAN PATENT SPECIFICATION

(11) **EP 0 044 669 B1**
(45) Date of publication and mention of the grant of the patent: **06.04.1988**
(21) Application number: 81303130.9
(22) Date of filing: 09.07.1981
(51) Int. Cl.: C22B 1/245, C22B 1/24

(54) **Self-reducing iron oxide agglomerates**
Selbstgehendes stückiges Eisenoxid
Agglomérés d'oxyde de fer auto-réductibles

(30) Priority: 21.07.1980 US 170643
(43) Date of publication of application: 27.01.1982
(73) Proprietor: BOARD OF CONTROL OF MICHIGAN TECHNOLOGICAL UNIVERSITY, Houghton, Michigan 49931 (US)
(72) Inventor: Goksel, Mehmet Adnan, Houghton Michigan 49931 (US)
(74) Representative: Taylor, Derek George

(56) References cited:
- AU-A- 425 513
- DE-A- 1 583 942
- DE-A- 2 517 543
- DE-B- 1 243 880
- US-A- 2 793 109
- US-A- 2 806 779
- US-A- 3 264 092
- US-A- 3 895 088

## Description

This invention relates to a process for producing self-reducing agglomerates from finely-divided, iron ore concentrates.

It is known to form finely-divided, iron oxide-containing materials, such as iron ore concentrates and steel plant waste dusts, into pellets containing internal carbon for the purpose of accelerating the rate of reduction of the iron oxide to metallic iron when the pellets are charged to a steel making furnace. Such processes are exemplified in United States Patent Specifications 2,793,109 (Huebler et al), 2,806,779 (Case), 3,264,092 (Ban), 3,333,951 (Ban), 3,386,816 (English), 3,770,416 (Goksel) and 3,938,987 (Ban) and Canadian Patent 844,592 (Volin et al).

It is generally recognized that in hitherto proposed processes the presence of a carbonaceous material in an amount sufficient to reduce all the iron oxide to metallic iron tends adversely to affect crush resistance or compressive strength of the pellets. In this regard, United States Patent Specifications 2,806,779 and 3,264,092 teach the use of an agglomerating type coal and then heating the pellets to a temperature of about 1600-2300°F to distill destructively the coal and thereby produce a char bond for the pellets. United States Specification 3,938,987 teaches that, when non-agglomerating coals, such as lignite, sub-bituminous coals, anthracite coal and coke breeze, are used at the carbonaceous material, the amount must be about 40-80% of that required to reduce iron oxide to metallic iron in order to produce pellets having adequate strength for use in a steel making furnace. United States Patent Specification 3,386,816 teaches that pellets containing as little as 8% coke have a compressive strength of 26 kg which is generally considered unacceptably low for use in most steel making processes.

The problem to be solved by the invention is to provide a low cost process for forming finely-divided, iron ore concentrates into hardened agglomerates containing an amount of carbonaceous material at least sufficient to reduce all the iron oxide to metallic iron and yet having high compressive strengths.

The problem is solved in accordance with the invention, in that the following steps are employed:
(a) preparation of a moistened starting mixture including the iron ore concentrates, a finely-divided natural or pyrolyzed carbonaceous material having a volatile matter (on dry basis) content of about 20% by weight or less in an amount at least sufficient to reduce all the iron oxide in the concentrates to metallic iron, about 1 to about 30% by weight of a finely-divided bonding agent such as the oxides, hydroxides, or carbonates of calcium and magnesium, or mixtures thereof, and 0 to up to about 3% by weight of a finely-divided siliceous material, as available Si0₂ capable of reacting with said bonding agent to form silicate or hydrosilicate bonds therewith with the total available Si0₂ in said mixture being at least 0.5 by weight, the weight percentages being based upon the total weight of the dry solids in said mixtures;
(b) allowing said mixture to stand without the addition of moisture for a time period sufficient for a substantial proportion of the free internal moisture in the pores of said carbonaceous material to migrate to the surface thereof;
(c) forming discrete green agglomerates from said starting mixture;
(d) drying said green agglomerates to a moisture content of about 5% by weight or less; and
(e) hydrothermally hardening said green agglomerates by contacting them with steam at a temperature of about 100 to 250°C for a time period sufficient for said bonding agent to form silicate or hydrosilicate bonds with the available Si0₂ and produce hardened and integrally bonded masses.

Previously proposed hydrothermally-hardened, iron oxide agglomerates containing carbonaceous materials, having a high volatile matter content, in an amount sufficient to reduce all the iron oxide to metallic iron exhibit crush resistance or compressive strengths which are unacceptably low for many uses. Quite unexpectedly, it has been found that the compressive strengths of such agglomerates can be increased significantly by using natural or pyrolyzed carbonaceous materials having a volatile matter (on a dry basis) content of about 20% by weight or less.

More specifically, the process of invention includes the steps of preparing a moistened mixture of finely divided iron ore concentrates, a finely-divided, natural or pyrolyzed carbonaceous material having a volatile matter (on dry basis) content of about 20% by weight or less in an amount at least sufficient to reduce all the iron oxide to metallic iron, about 1 to about 30 weight % of a bonding agent selected from a group consisting of oxides, hydroxides and carbonates of calcium and magnesium and mixtures thereof, and 0 to about 3 weight % of a siliceous material (as available Si0₂); forming the resulting mixture into discrete green agglomerates; and hydrothermally hardening the green agglomerates by contacting them with steam for a time period sufficient to form them into hardened, integral bonded masses.

The process is particularly suitable for producing high strength agglomerates from iron ores, such as haematite and magnetite, preferably in the form of high purity ores or concentrates containing about 45-70% iron and the balance gangue and oxide.

A starting mixture is first prepared by thoroughly blending together an iron ore concentrate, a carbonaceous material, a bonding agent, a siliceous material and a sufficient amount of water to form a moistened mixture capable of being formed into discrete agglomerated masses or pellets.

The carbonaceous material can be either naturally occurring or pyrolyzed so long as it has a volatile matter (on dry basis) content of about 20% by weight or less, preferably about 10 weight % or less. Pyrolyzed carbonaceous materials generally are preferred because .of their lower volatile content.

Representative suitable natural carbonaceous materials include low volatile anthracite coal, graphite and the like.

The term "pyrolyzed carbonaceous material" as used herein means a solid product produced by heating a naturally occurring, high carbonaceous material to elevated temperatures in the absence of oxygen to drive off a substantial portion of the volatile matter, primarily organic matter. Representative suitable pyrolyzed carbonaceous materials include chars produced from non-coking bituminous, sub-bituminous and anthracite coals, lignite char, wood char, coke produced from bituminous coal, coke breeze, petroleum and coal tar pitch, and mixtures thereof. Of these, bituminous coal char, lignite char and coke breeze are preferred because of their lower cost.

Suitable bonding agents include the oxides, hydroxides, and carbonates of calcium and magnesium and mixtures thereof. Burned lime (CaO) and hydrated lime (Ca(OH)₂) are preferred because, in addition to functioning as a bonding agent, they can assist in slag formation and sulfur removal when the agglomerates are used in a steel making process.

The amount of bonding agents used is about 0.1 to about 30% by weight, based on the total weight of the dry solids in the starting mixture. When less than about 0.1 weight % is used, the hardened pellets do not have sufficient crush resistance or compressive strength to withstand the loads normally imposed thereon during handling, storage and transportation. On the other hand, amounts of the bonding agents in excess of about 30% by weight do not appreciably increase the compressive strengths, can dilute the concentration of iron oxide in the final agglomerates to an undesirable level and can cause formation of excessive amounts of slag during melting. The preferred amount of bonding agent is about 2 to about 10% by weight.

If the iron ore concentrate contains an appreciable amount (e.g., about 0.5% by weight or more) of available Si0₂ capable of reacting with the bonding agent to formed silicate or hydrosilicate bonds therewith during the conditions of hydrothermal hardening, hardened pellets having compressive strengths up to about 90 kg can be obtained without adding a siliceous material to the starting mixture. For higher purity iron ore concentrates containing relatively small amounts of available Si0₂, an amount of natural or artificial siliceous material containing up to 3% by weight available Si0₂, based on the total weight of the dry solids, is added to the starting mixture. The total available Si0₂ in the mixture, whether as part of the iron ore concentrate or added with the siliceous material, should be at least 0.5% by weight.

Representative suitable siliceous materials include finely ground quartz, silica sand, bentonite, diatomaceous earth, fuller's earth, sodium, calcium magnesium, and aluminum silicates, pyrogenic silica, various hydrated silicas and mixtures thereof. Of these, finely ground quartz and silica sand are preferred.

In addition to the bonding agent and the siliceous material, other strengthening additives can be included in a starting mixture to further increase the strength of the hardened agglomerates. For example, oxides, hydroxides, carbonates, bicarbonates, sulfates, bisulfate, and borates of alkali metals (e.g. potassium and sodium) and mixtures thereof can be added in amounts ranging to about 3% by weight. Of these, sodium hydroxide, sodium carbonate, and sodium bicarbonate are preferred. Furthermore, quaternary ammonium hydroxides, quaternary ammonium chlorides or quaternary amines or mixtures thereof may be used as strengthening additives. The presence of some of these strengthening additives might be considered undesirable when the hardened agglomerates are used as a charge for blast furnaces. In those cases, such additives can be omitted without significantly reducing the strength of the agglomerates. When used, the preferred amount of the strengthening additives is about 0.15 to about 1% by weight.

The amount of water included in the starting mixture varies, depending on the physical properties of the materials and the particular agglomeration technique employed. For example, when a pelletizing process employing a balling drum or disc is used to form spherical pellets, the total amount of water in the moistened starting mixture generally should be about 5 to about 20% by weight, preferably about 10 to about 15% by weight. On the other hand, when a briquetting press is used, the amount of water in the moistened starting moisture generally should be about 3 to about 15% by weight, preferably from about 5 to about 10% by weight.

The average particle size of the various solid materials included in the starting mixture generally can range from about 10 to about 325 mesh with all preferably being less than about 200 mesh. Particle sizes coarser than about 100 mesh make it difficult to obtain a homogeneous mixture of the constituents and, in some cases, produce insufficient surface area to obtain the requisite high strength bond in the hardened agglomerates. Also, it is difficult to form pellets from mixtures containing coarser particles. Preferably, at least half of all solid materials in the starting mixture have an average particle size less than about 200 mesh for pelletizing. Briquettes can be produced with coarser particles.

Many low volatile, naturally occurring and pyrolyzed carbonaceous materials have small capillary-like pores or cavities which tend to absorb water during the mixing step. This free internal moisture tends to be converted to steam during the hydrothermal hardening step, causing a reduction in the compressive strength and sometimes cracking or bursting when excessive amounts are present in the pores or cavities. This can be minimized by allowing the moistened mixture to rest or stand a sufficient time for a substantial portion of the free internal moisture in the carbonaceous material to migrate from the pores or cavities to the surface.

The time and conditions for this holding or standing step can vary considerably depending primarily on the particular type of carbonaceous material and bonding agent being used. Removal of excess internal moisture from the pores or cavities in the carbonaceous material can be accelerated by heating the moistened mixture to an elevated temperature. When burned lime and/or magnesium oxide is used as the bonding agent, they react with the moisture present to form hydrates. This exothermic hydration reaction tends to accelerate migration of the free internal moisture to the particle surface, resulting in a shortening of the standing time required without external heating.

As a general guide, the moistened mixture, prior to agglomeration, is allowed to stand for about 0.5 to about 48 hours, preferably about 2 to about 3 hours, at a temperature of about 60 to about 90°C. Higher temperatures and pressures can be used, but are less desirable because of the higher operational costs. When burned lime or magnesium oxide is used as the bonding agent, the moistened mixture preferably is placed in a closed, thermally insulated container to take advantage of the exothermic hydration reaction.

The moistened mixture is next formed into green agglomerates of the desired size and shape for the intended end use by a conventional agglomeration technique, such as molding, briquetting, pelletizing, extruding and the like. Pelletizing with a balling disc or drum is preferred because of the lower operating costs.

When in the form of spherical pellets, the green agglomerates generally have a diameter of about 5 to about 25 mm, preferably about 10 to about 20 mm. When briquetting is used, the agglomerates preferably are in a spherical-like or egg shape and have a major diameter ranging up to about 75 mm. Larger pellets and briquettes can be used if desired.

The crush resistance or compressive strength of the hardened agglomerates can be increased by drying the green agglomerates to a free moisture content of about 5% by weight or less, preferably about 3% by weight or less, prior to the hydrothermal hardening step. This drying can be accomplished by conventional means, such as by placing the green agglomerates in an oven or by blowing a heated gas thereover, using drying temperatures up to the decomposition temperature of the carbonaceous material. The time required to reduce the free moisture content to about 5% by weight or less depends upon the drying temperatures used, the moisture content of the green agglomerates, flow rate of the drying gas, the level to which the moisture content is reduced, size and shape of the green agglomerates, etc.

The green agglomerates are introduced into a reaction chamber or pressure vessel, such as an autoclave, wherein they are heated to an elevated temperature in the presence of moisture to effect a hardening and bonding of the individual particle into an integral, high strength mass. The compressive strength of the hardened agglomerates produced by this hydrothermal hardening step depends to some extent upon the temperature, time, and moisture content of the atmosphere use.

The application of heat to the green agglomerates can be achieved by any one of a number of methods. The use of steam is preferred because it simultaneously provides a source of heat and moisture necessary for the hydrothermal reaction. Either saturated steam or substantially saturated steam can be used. Superheated steam tends to produce hardened agglomerates having reduced strengths. Therefore, steam at temperatures and pressures at or close to that of saturated steam is preferred. Temperatures generally ranging from about 100 to about 250°C, preferably 200 to about 225°C, can be satisfactorily employed to achieve the desired hardening of the green agglomerates within a reasonable time period.

Autoclaving pressures substantially above atmospheric pressure are preferred in order to decrease the hardening time and to improve the strength of the hardened agglomerates. Generally, economic conditions dictate that the maximum pressure should not exceed about 35 atmospheres and a pressure of about 10 to about 25 atmospheres is preferred.

The retention time of the pellets in the reaction chamber or pressure vessel depends upon several process variables, such as pressure, temperature, and atmosphere of the chamber, size and composition of the pellets, etc. In any case, this time should be sufficient for the bonding agent to form silicate and/or hydrosilicate bonds in the available Si0₂ and bond the individual particles into a hardened, high strength condition. When higher temperatures and pressures are used, the time for the hydrothermal hardening generally is about 5 minutes to about 15 hours, preferably about 30 to about 60 minutes.

The hardened agglomerates are removed from the reacting chamber and, upon cooling, are ready for use. The hot, hardened agglomerates usually contain up to about 1.5% free moisture and have compressive strength characteristics suitable for most uses. The compressive strength of the hardened agglomerates can be increased by rapidly drying them, preferably immediately after removal from the reaction chamber and before appreciable cooling has occurred, to remove substantially all of the free moisture therefrom. This drying can be accomplished in a convenient manner.

The minimum compressive strength of hardened agglomerates produced by the process of the invention varies depending on the size of the agglomerate. For example, spherical pellets with a diameter of 12-15 mm have a compressive strength of at least 45 kg and those with a diameter of about 30 mm have a compressive strength in the neighbourhood of about 90 kg or more.

Without further elaboration, it is believed that one skilled in the art, using the preceding description, can utilize the invention to its fullest extent. The following example is presented to illustrate the invention and should not be construed as a limitation thereto.

### Example

A series of tests was run to evaluate the crush resistance or compressive strength of hardened magnetite pellets containing different types of carbonaceous materials in amounts sufficient to reduce all the iron oxide to metallic iron. The ingredients making up the starting mixture were blended together in a roller or intensive mixer for a sufficient time to obtain a uniformly moistened blend. Green, spherically- shaped pellets (15 mm) were prepared from the mixtures in a conventional balling device. The green pellets were dried to a moisture content of about 0-3% by weight and then placed in a high pressure steam autoclave. The autoclave was heated and maintained at a temperature of 210°C and a pressure of 22 atm for one hour. After cooling, the compressive strength of the pellets was measured with a Dillon tester. Results from these tests are summarized in Table I.

From these results, it can be seen that pellets containing a carbonaceous material having a low volatile matter content (anthracite) or which was pyrolyzed (bituminous coal char, lignite char and coke), had compressive strengths in excess of 45 kg. Whereas those containing a carbonaceous material having a high volatile matter content (bituminous coal and lignite) had substantially lower compressive strengths. The use of chars from non-coking bituminous coal, lignite and other low grade carbonaceous materials is particularly advantageous because of the low cost of these materials and the volatiles driven off during the pyrolyzing process can be burned and used as a heat source.

## Claims

1. A process for producing self-reducing agglomerates from finely-divided, iron ore concentrates comprising the steps of
(a) preparing a moistened starting mixture including the iron ore concentrates, a finely-divided natural or pyrolyzed carbonaceous material having a volatile matter (on a dry basis) content of about 20% by weight or less in an amount at least sufficient to reduce all the iron oxide in the concentrates to metallic iron, about 1 to about 30% by weight of a finely-divided bonding agent such as the oxides, hydroxides, or carbonates of calcium and magnesium, or mixtures thereof, and 0 to up to about 3% by weight of a finely-divided siliceous material, as available Si0₂ capable of reacting with said bonding agent to form silicate or hydrosilicate bonds therewith with the total available Si0₂ in said mixture being at least 0.5% by weight, the weight percentage being based upon the total weight of the dry solids in said mixtures;
(b) allowing said mixture to stand without the addition of moisture for a time period sufficient for a substantial proportion of the free internal moisture in the pores of said carbonaceous material to migrate to the surface thereof;
(c) forming discrete green agglomerates from said mixture as prepared in step (b);
(d) drying said green agglomerates to a moisture content of about 5% by weight or less; and
(e) hydrothermally hardening said green agglomerates by contacting them with steam at a temperature of about 100 to 250° for a time period sufficient for said bonding agent to form silicate or hydrosilicate bonds with the available Si0₂ and produce hardened and integrally bonded masses.

2. A process according to claim 1 wherein volatile matter content of said carbonaceous material is about 10% by weight or less.

3. A process according to claim 2 wherein step (b) is carried out at a temperature of about 60 to about . 90°C for a time period of about 0.5 to about 48 hours.

4. A process according to claim 2 wherein said moistened mixture includes up to about 3% by weight, based on the total weight of the dry solids in said mixture, of a strengthening additive including the oxides, hydroxides, carbonates, bicarbonates, sulfates, bisulfates, or the borates of the alkali metals, quaternary ammonium hydroxides, quaternary ammonium chlorides, or quaternary ammonium amines, or mixtures thereof.

5. A process according to claim 4 wherein said strengthening additive is sodium hydroxide, sodium carbonate, or sodium bicarbonate.

6. A process according to any one of claims 1 to 5 wherein said siliceous material is silica.

## Patentansprüche

1. Verfahren zur Herstellung von selbstreduzierenden Agglomeraten aus fein zerteilten Eisenerzkonzentraten, das die folgenden Stufen umfaßt:
(a) Herstellen einer angefeuchteten Ausgangsmischung, einschließlich der Eisenerzkonzentrate, eines fein zerteilten natürlichen oder pyrolisierten kohlenstoffhaltigen Materials mit einem Gehalt an flüchtigen Stoffen (auf Trockenbasis) von etwa 20 Gew.-% oder weniger in einer Menge, die wenigstens ausreichend ist, um das ganze Eisenoxid in den Konzentraten zu metallischem Eisen zu reduzieren, etwa 1 bis etwa 30 Gew.-% eines fein zerteilten Bindemittels, wie die Oxide, Hydroxide oder Carbonate von Calcium und Magnesium oder Mischungen daraus, und 0 bis zu etwa 3 Gew.-% eines fein zerteilten siliciumhaltigen Materials, als erhältliches Si0₂, das mit dem Bindemittel reagieren kann, um Silicat- oder Hydrosilicatbindungen damit zu bilden, wobei das gesamte erhältliche Si0₂ in der Mischung wenigstens 0,5 Gew.-% beträgt, wobei der Gew.-Prozentsatz auf das Gesamtgewicht der trockenen Feststoffe in der Mischung bezogen ist;
(b) Stehenlassen der Mischung ohne Zugabe von Feuchtigkeit über einen Zeitraum, der ausreichend ist, damit ein wesentlicher Anteil der freien inneren Feuchtigkeit in den Poren des kohlenstoffhaltigen Materials an die Oberfläche wandert;
(c) Bilden von diskreten bzw. getrennten grünen Agglomeraten aus der in der Stufe (b) hergestellten Mischung;
(d) Trocknen der grünen Agglomerate auf einen Feuchtigkeitsgehalt von etwa 5 Gew.-% oder weniger und
(e) hydrothermales Aushärten der grünen Agglomerate, indem diese mit Dampf bei einer Temperatur von etwa 100 bis 250° in Kontakt gebracht werden über einen Zeitraum, der für das Bindemittel ausreichend ist, um Silicat- oder Hydrosilicatbindungen mit dem erhältlichen Si0₂ zu bilden und ausgehärtete und integriert gebundene Massen herzustellen.

2. Verfahren nach Anspruch 1, worin der Gehalt an flüchtigen Stoffen in dem kohlenstoffhaltigen Material etwa 10 Gew.-% oder weniger beträgt.

3. Verfahren nach Anspruch 2, worin die Stufe (b) bei einer Temperatur von etwa 60 bis etwa 90°C über einen Zeitraum von etwa 0,5 bis etwa 48 Stunden durchgeführt wird.

4. Verfahren nach Anspruch 2, worin die angefeuchtete Mischung bis zu etwa 3 Gew.-%, bezogen auf das Gesamtgewicht der trockenen Feststoffe in der Mischung, eines Verstärkungsadditivs, einschließlich der Oxide, Hydroxide, Carbonate, Bicarbonate, Sulfate, Bisulfate oder Borate von Alkalimetallen, quaternäre Ammoniumhydroxide, quaternäre Ammoniumchloride oder quaternäre Ammoniumamine oder Mischungen daraus, einschließt.

5. Verfahren nach Anspruch 4, worin das Verstärkungsadditiv Natriumhydroxid, Natriumcarbonat oder Natriumbicarbonat ist.

6. Verfahren nach einem der Ansprüche 1 bis 5, worin das siliciumhaltige Material Siliciumdioxid ist.

## Revendications

1. Un procédé pour la production d'agglomérés autoréductibles à partir de concentrés de minerais de fer finement divisés comprenant les étapes de
(a) préparation d'un mélange de départ humidifié comprenant les concentrés de minerais de fer, une matière carbonée naturelle ou pyrolysée finement divisée ayant une teneur en matière volatile (en poids sec) d'environ 20% en poids ou moins, en quantité au moins suffisante pour réduire tout l'oxyde de fer dans les concentrés en fer métallique, environ 1 à environ 30% en poids d'un agent liant finement divisé tel que les oxydes, hydroxydes ou carbonates de calcium et de magnésium ou leurs mélanges et de 0 jusqu'à environ 3% en poids d'une matière siliceuse finement divisée, calculée en Si0₂ disponible capable de réagir avec ledit agent liant pour former avec celui-ci des liaisons silicates ou hydrosilicates, le Si0₂ total disponible dans ledit mélange étant d'au moins 0,5% en poids, les pourcentages en poids étant rapportés' au poids total des solides secs dans lesdits mélanges;
(b) repos dudit mélange sans addition d'humidité pendant une durée suffisante pour qu'une proportion substantielle de l'humidité interne libre dans les pores de ladite matière carbonée migre à la surface de celle-ci;
(c) formation d'agglomérés verts distincts à partir dudit mélange;
(d) séchage desdits agglomérés verts jusqu'à une teneur en humidité d'environ 5% en poids ou moins; et
(e) durcissement hydrothermique desdits agglomérés verts par mise en contact avec de la vapeur à une température d'environ 100 à 250°C pendant une durée suffisante pour que ledit agent liant forme des liaisons silicates ou hydrosilicates avec le Si0₂ disponible et produise des masses durcies et intégralement liées.

2. Un procédé selon la revendication 1, dans lequel la teneur en matière volatile de ladite matière carbonée est d'environ 10% en poids ou moins.

3. Un procédé selon la revendication 2, dans lequel l'étape (b) est mise en oeuvre à une température d'environ 60 à environ 90°C pendant une durée d'environ 0,5 à environ 48 heures.

4. Un procédé selon la revendication 2, dans lequel ledit mélange humidifié contient jusqu'à environ 3% en poids, par rapport au poids total des solides secs dans ledit mélange, d'un additif de renforcement comprenant les oxydes, hydroxydes, carbonates, bicarbonates, sulfates, bisulfates ou borates des métaux alcalins, les hydroxydes d'ammonium quaternaires, chlorures d'ammonium quaternaire ou dérivés quaternaires organiques d'amines ou leurs mélanges.

5. Un procédé selon la revendication 4, dans lequel ledit additif de renforcement est l'hydroxyde de sodium, le carbonate de sodium ou le bicarbonate de sodium.

6. Un procédé selon l'une quelconque des revendications 1 à 5, dans lequel ladite matière siliceuse est la silice.
